

## UNITED STATES PATENT OFFICE.

ARTHUR W. BURWELL, OF NIAGARA FALLS, NEW YORK, ASSIGNOR TO ALOX CHEMICAL CORPORATION, OF NEW YORK, N. Y., A CORPORATION OF NEW YORK

## ATOMIZABLE MOBILE FUEL PRODUCT.

No Drawing.

Application filed March 2, 1927. Serial No. 172,214.

This invention relates to an atomizable mobile fuel product of the type consisting essentially of finely divided solid fuel dispersed in a normally liquid fuel and held 5 in a state of substantially stable suspension therein by means of a stabilizing agent, and to an economical process of making the same.

The many obvious advantages to be derived from the use of a mobile fuel composition having a higher fuel value per unit volume than fuel oil alone previously have led to attempts to utilize powdered solid fuel mixed with, or dispersed in, liquid fuel. 10 It was early found that finely divided solid fuel (e. g., powdered coal) settles out of an intimate admixture of the same with fuel oil within a very short period of time (i. e., about from four to seven days), and results 15 in the deposition of a hard solid mass, consisting essentially of the finely divided solid fuel, which can be re-mixed with the fuel oil only by resorting to laborious and uneconomical mechanical agitation means. 20 Previous investigators have attempted to stabilize the suspension of finely divided solid fuel in liquid fuel by the admixture therewith of rosin compounds, lime-rosin grease, coal distillates, gelatin, albumen, 25 soaps and the like. Relatively stable suspensions have been prepared by the use of one or more of these stabilizing agents in the powdered solid fuel-fuel oil mixtures, particularly in those cases where the solid 30 fuel particles have been reduced to a substantially colloidal size in the presence of the liquid fuel and of the stabilizing agent. Such fluid fuel compositions, while exhibiting remarkable colloid-like properties with 35 regard to the stability of the suspensions, are not of commercial use because of the high costs entailed in their preparation. 40

An object of the invention is to provide an atomizable mobile fuel product having the said desirable characteristics, and which may be prepared in such an economical manner that the product may compete commercially with powdered coal.

The invention is based upon my discovery 50 of the fact that a petroleum soluble, non-aqueous mobile colloidal gel may be produced from a normally liquid petroleum hydrocarbon mixture such as the petroleum distillates commonly used as fuel and known 55 generally as "fuel oils", by dissolving there-

in an alkali metal salt of a saponifiable, organic acidic product obtained by the controlled oxidation of a normally liquid aliphatic hydrocarbon, and that finely divided solid fuel, when dispersed in said petroleum soluble, non-aqueous mobile colloidal gel, is held therein in a state of substantially stable suspension. 60

It has been found that by the practicing 65 of my invention the solid fuel (e. g., coal) need not be reduced in particle size to the colloid-like state in order to effect the production of a stable mobile fuel product therefrom, it being necessary only that the solid fuel particles be of a sufficient degree 70 of fineness so that they readily may pass through the passages of the fuel burning apparatus without danger of clogging,—i. e., of about the particle size of about from 100 to 200 mesh. 75

The petroleum soluble, non-aqueous, mobile, colloidal gel serving as the suspension agent for the finely divided solid fuel is prepared, as hereinbefore mentioned, by dissolving in a normally liquid petroleum hydrocarbon mixture (e. g., fuel oil) an alkali metal salt of a saponifiable, organic acidic product obtained by the controlled oxidation of a normally liquid aliphatic hydrocarbon or hydrocarbon mixture. The said alkali metal salt does not form with the fuel oil a true solution, but forms a mobile colloidal solution, or gel which is sufficiently fluid to permit being pumped easily. 80 85

There follows a detailed description of 90 the preferred process of making the petroleum soluble, non-aqueous mobile colloidal gel, it being understood that the invention is not limited to the specific materials, proportions and conditions hereinafter to be set out, which are understood to be exemplary: 95

Although the organic acidic products obtained by the controlled liquid-phase oxidation of hydrocarbons or mixtures thereof generally, under such conditions as to obtain water-insoluble, saponifiable, organic acidic products, are adapted for use in the preparation of the aforesaid alkali metal salts, I prefer, for purely economical reasons, to employ the organic acidic products from the cheapest fuel oil available,—for instance, the fuel oil known as "36 to 40° Baumé fuel distillate." When a petroleum distillate of this type and character, in the 100 105 110

liquid phase, is contacted with an oxygen-containing gas such as, for example, air, at a temperature of from about 120° to about 140° C. and at a pressure of from about 150 pounds to about 350 pounds per square inch,—say 250 pounds per square inch,—there is formed a reaction mixture comprising water-soluble acids of relatively low molecular weight,—such as, for example, formic acid,—unsaponifiable oxygenated organic compounds, unoxidized petroleum hydrocarbons, and a water-insoluble, saponifiable, organic, acidic product which is wholly or partly soluble in the petroleum hydrocarbon mixture. In the oxidation step, the oxidation per se may be initiated by the presence in the petroleum distillate of a small amount of an oxidizing catalyst, such as a compound of manganese, copper or iron, say manganese stearate, amounting to about 0.1 percent of the weight of the petroleum distillate. Or, the oxidation may with equal facility be initiated by providing as the charge of raw material to undergo oxidation a mixture comprising about equal parts by weight or volume of fresh petroleum distillate and unoxidized petroleum hydrocarbons from a previously treated charge.

30 The oxidation step preferably is terminated at a point where incipient formation of oxidation products insoluble in the reaction mixture commences; e. g. at a point where the partially oxidized mass contains 35 from about 25 to about 30 percent of saponifiable acidic products as titrated for a molecular weight of 280. These saponifiable acidic products consist essentially of simple aliphatic carboxylic acids derived from 40 the aliphatic hydrocarbons which made up the bulk of the petroleum distillate starting material. They are insoluble in water but soluble in the petroleum distillate.

45 For obtaining the desired saponifiable organic acid product, the above-described reaction mixture is washed with water, thereby removing the water-soluble acids, and the resulting washed product is treated with an aqueous solution of a caustic alkali in quantity sufficient to saponify the acid compounds constituting the said water-insoluble, saponifiable organic acidic product. The reaction mixture resulting from the treatment with caustic alkali solution is diluted 55 with water,—in order to throw out of solution any dissolved unsaponified material, whereby there are formed, upon standing, a supernatant non-aqueous oily layer comprising unoxidized material and unsaponifiable 60 products of oxidation, and a subnatant aqueous layer comprising a solution of the alkali metal salt of the saponifiable organic acidic product.

65 The subnatant aqueous layer is carefully separated from the supernatant oily layer

and is dehydrated to a perfectly dry mass. The dehydration may be effected, without danger of charring, by subjecting the aqueous solution to evaporation treatment at a temperature of about 150° C., but I prefer 70 to effect the dehydration by mixing with the soap solution an equal quantity of fuel oil and subjecting the mixture to heat treatment at a temperature of about 120° C. In the latter procedure the mixture remains fluid 75 throughout the dehydration and the water content may be driven off much more freely than from the soap solution alone; also, the soap solution is less prone to decomposition. To the solution of non-aqueous soap in fuel 80 oil obtained by the above procedure, I add a sufficient quantity of fuel oil to yield the desired concentration of soap in the mixture.

85 The dehydrated mass, resulting from the above described treatment and consisting essentially of the alkali metal salt of the saponifiable organic acidic product obtained by the controlled oxidation of a normally liquid petroleum hydrocarbon mixture, is found to be soluble in ordinary fuel oil to the production of a colloidal solution. Said colloidal solution has strong gel-forming tendencies, it being a fact that the presence of 90 only about 1 to 2 parts by weight of said alkali metal salt in 100 parts by weight of the solution effects the production of a colloidal gel which, while sufficiently fluid to be pumped easily, is capable of holding 95 therein powdered coal having a particle size of about from 100 to 200 mesh in a state of stable suspension for a prolonged period of time, i. e., a month or more. The conversion of the fuel oil from a liquid state to 100 the state of a mobile gel apparently does not detract from its fuel value. Powdered coal of about from 100 to 200 mesh is introduced into said fuel oil gel and suspended 105 therein by simple mechanical agitation.

110 The relative proportion of powdered coal to fuel oil gel may be varied within wide limits, it being possible to prepare a stable mobile fuel product therefrom containing equal parts by weight of the coal and the gel. It is to be noted that the relative proportions of the coal and the gel may be so selected as to obtain an atomizable mobile fuel product having a predetermined thermal value and density per unit of volume. For example, the powdered coal and the fuel oil gel may be brought together in such proportions as to yield a product ranging in weight between 8 and 12 pounds per gallon (231 cubic inches) of space and having, especially in the more dense compositions, a thermal value much greater than that of an equal volume of fuel oil or of powdered coal alone.

115 It is a remarkable fact that, although on 120 long standing there may occur some strati- 125

fication into layers having different proportions of solid fuel and fuel oil gel, these layers may be re-mixed easily, and the deposition of an objectionable amount of sediment does not occur.

This application contains subject matter which is common to my copending applications Ser. No. 588,073, filed Sept. 13, 1922, and Ser. No. 642,638, filed May 31, 1923, respectively.

I claim:

1. Process which comprises producing a petroleum soluble, non-aqueous mobile colloidal gel from a normally liquid petroleum hydrocarbon mixture and suspending in said non-aqueous mobile colloidal gel finely divided solid fuel.

2. Process of producing an atomizable mobile fuel product involving the suspension of finely divided solid fuel in a liquid fuel in the presence of a stabilizing agent, characterized in that there is used as the stabilizing agent a petroleum soluble, alkali metal salt of a saponifiable organic acidic product substantially identical with that obtained by contacting an oxidizing gas with a normally liquid petroleum hydrocarbon mixture, in liquid phase, at reacting temperatures and at a pressure greater than atmospheric pressure.

3. Process of producing an atomizable mobile fuel product which comprises dissolving in a normally liquid petroleum hydrocarbon mixture a petroleum soluble, neutral alkali metal salt of a saponifiable organic acidic product substantially identical with that obtained by contacting an oxidizing gas with a normally liquid petroleum hydrocarbon mixture, in liquid phase, at reacting temperature and at a pressure greater than atmospheric, whereby there is obtained a mobile colloidal gel of said normally liquid petroleum hydrocarbon mixture, and suspending in said mobile colloidal gel finely divided solid fuel.

4. As a new atomizable mobile fuel product, a substantially stable suspension of finely divided solid fuel in a non-aqueous, mobile, colloidal gel comprising a normally liquid petroleum hydrocarbon mixture and a petroleum soluble alkali metal salt of a saponifiable organic acidic product substantially identical with that obtained by con-

tacting an oxidizing gas with a normally liquid petroleum hydrocarbon mixture, in liquid phase, at reacting temperature and at a pressure greater than atmospheric pressure.

5. As a new atomizable mobile fuel product, a substantially stable suspension of finely divided solid fuel in a non-aqueous mobile, colloidal gel comprising a solution containing about 98 parts by weight of a normally liquid petroleum hydrocarbon mixture and about 2 parts by weight of a petroleum soluble alkali metal salt of a saponifiable organic acidic product substantially identical with that obtained by contacting an oxidizing gas with a normally liquid petroleum hydrocarbon mixture, in liquid phase, at reacting temperature and at a pressure greater than atmospheric pressure.

6. As a new atomizable mobile fuel product, a composition comprising about 100 parts by weight of powdered coal having a particle size of about from 100 to 200 mesh suspended in a fuel oil gel consisting of about 98 parts by weight of a normally liquid fuel oil and about 2 parts by weight of a petroleum soluble alkali metal salt of a saponifiable organic acidic product substantially identical with that obtained by contacting an oxidizing gas with a normally liquid petroleum hydrocarbon mixture, in liquid phase, at reacting temperature and at a pressure greater than atmospheric pressure.

7. Process of producing an atomizable mobile fuel product which comprises dissolving in a normally liquid petroleum hydrocarbon mixture an alkali metal salt of a saponifiable organic acidic product obtained by the controlled oxidation of normally liquid petroleum hydrocarbons.

8. As a new atomizable mobile fuel product, a substantially stable suspension of finely divided solid fuel in a non-aqueous, mobile, colloidal gel, comprising a solution containing a normally liquid petroleum hydrocarbon mixture and an alkali metal salt of a saponifiable organic acidic product obtained by the controlled oxidation of a normally liquid petroleum hydrocarbon mixture.

In testimony whereof, I affix my signature.  
ARTHUR W. BURWELL.